

Jan. 4, 1938.

L. DAVIS

2,104,025

DECALCOMANIA PAPER

Filed Aug. 23, 1934



*Fig. 1*

*Fig. 2.*



INVENTOR:  
*Lewis Davis*

BY  
*J. W. McCready*,  
his ATTORNEY.

## UNITED STATES PATENT OFFICE

2,104,025

## DECALCOMANIA PAPER

Lewis Davis, Worcester, Mass., assignor to Mc-Laurin-Jones Co., Brookfield, Mass., a corporation of Massachusetts

Application August 23, 1934, Serial No. 741,121

9 Claims. (Cl. 41—33)

This invention relates to decalcomanias and is more especially concerned with the papers on which decalcomania designs are printed.

In applying such designs to some articles of work, such as water absorbent bodies and especially wood veneers, the use of the necessary quantity of water required to separate the backing sheet from the decalcomania film is highly objectionable because it tends to warp the veneer and make it difficult to properly register or abut the edges of adjoining sheets. If, in addition, the veneer is to be applied to a body or core made of wood, or some other water absorbent material, which usually is the case, then the application of water is even more objectionable. This factor becomes especially important in applying such designs to large surfaces such, for example, as wood paneling.

The present invention deals with the problem presented by these conditions and it aims to devise a decalcomania paper which will avoid these objections.

The nature of the invention will be readily understood from the following description when read in connection with the accompanying drawing, and the novel features will be particularly pointed out in the appended claims.

In the drawing,

Figure 1 is a perspective view of a portion of a sheet of decalcomania paper embodying features of this invention; and

Fig. 2 is a vertical, sectional view on a large scale of a portion of the sheet shown in Fig. 1.

The product shown in the drawing comprises a backing sheet 1 of paper carrying on one face thereof two superposed coats of waterproof material, (the term "waterproof" being used in its common, rather than its strictly scientific, sense), the respective coats being designated at 2 and 3. This sheet may be of any suitable character, such, for example, as the unsized backing papers commonly used heretofore in decalcomania papers, but in any event should be readily penetrable by the releasing solvent. The upper or outer coat 3 should have a smooth, uniform surface adapted to take decalcomania printing, while the under coat 2 acts both as a sizing to prevent the penetration of the upper coating material into the backing sheet during the manufacturing operations, and serves also to bond the outer coat to the backing sheet. A further highly desirable property in this under coat is that it shall possess a high degree of "slip" when wet with the releasing liquid or solvent in order to facilitate the separation of the decalcomania film from the

backing sheet 1. For some purposes it is desirable also to have coatings differentially soluble in non-aqueous solvents, or, in other words, to have each coating soluble in a solvent to which the other is highly resistant. But it is also important for most purposes that both coats be readily soluble in some non-aqueous solvent which is inexpensive, is readily obtainable, and which, therefore, can be used in effecting the release of the decalcomania film.

I have found that the foregoing requirements can be satisfied by making the outer coat of a resinous nature and the under coat of a rubbery character. The best material which I have so far discovered for the outer coat 3 is the synthetic resin known commercially as Cumar.

For the under coat I prefer to use rubber latex, although various other rubber compositions can be employed satisfactorily.

According to the preferred method, a small proportion of glue is added to the rubber latex in order to increase the adhesive properties of this material and thus to produce a better bond with the backing sheet. A typical formula consists of thirty parts of a good grade of the rubber latex of commerce, of the usual concentration, (having approximately 35% of solids), casein glue 2½ parts, water 40 parts, and ammonia 1 part. All of these proportions are by weight. A satisfactory casein glue mixture may be made by dissolving one part of casein in four parts of water and using any suitable alkali in a proportion of about 15% of the weight of the casein to assist in dissolving the latter ingredient. Other adhesives such as animal or fish glue, gum arabic, and the like, can be substituted for the casein.

The application of the glue and latex mixture to the paper may conveniently be made in the usual coating machinery. For most purposes an extremely thin coat only is required, say from one to two pounds of solid constituents to a ream of paper, the sheets measuring 20 x 24 inches. The thickness of this coating, however, can be varied to suit the requirements of individual situations by suitably controlling the consistency of the mixture. As above stated, this coating acts as a sizing to prevent the penetration of the second coating into the backing sheet.

After the first coat has been applied and allowed to dry it is calendered and then the outer Cumar 50 coat is put on. Cumar is known chemically as a coumarone-indene resin and may be defined as a mixture of para-coumarone, para-indene and the polymers of other hydrocarbons found in coal tar. It is a neutral resin produced from coal 55

tar distillates and is soluble in a considerable variety of common solvents such as gasoline and other petroleum distillates, carbon tetrachloride, ethyl and amyl acetates, and others. In preparing this coating material for application to the backing sheet, it should be borne in mind that the outer coating 3 must be very flat, smooth, and free from imperfections since the decalcomania design will be printed on this surface. For this reason it is desirable to associate suitable plasticizers with the Cumar resin and the solvents for it in order to produce a coating of the desired smoothness. Since the least expensive of the solvents for the Cumar consists of a petroleum distillate, it is ordinarily preferable to use this material. Assuming that in the final product the Cumar coat is to weigh four pounds to the ream, with sheets of the size above mentioned, a suitable composition may be composed of the following ingredients:

|                   | Grams |
|-------------------|-------|
| Cumar             | 814   |
| Ethyl acetate     | 424   |
| Butyl Cellosolve  | 12    |
| Dibutyl phthalate | 48.5  |
| Trolucoil         | 725   |

Of these constituents the chief solvent is the Trolucoil which is a petroleum distillate having a boiling range of from about 99° C. to 116° C. Other petroleum fractions, however, can be substituted for it. The ethyl acetate is a solvent aid. The dibutyl phthalate is a plasticizer, and the Butyl Cellosolve (ethylene glycol monobutyl ether) performs similar functions, acting as a leveling agent. The latter may, however, be omitted. This composition produces a very smooth satisfactory coating.

The paper so prepared is shipped to the decalcomania manufacturer who prints his design on the surface of the outer coat 3. The decalcomania so produced may be either of the ordinary transfer type or of the so-called "slide off" variety. After it has been applied to the work it is freed or released from the backing sheet by applying gasoline or some other suitable solvent to the surface of the backing paper, this solvent penetrating the paper readily and acting rapidly on the latex rubber under coat. As above stated, this coating is very thin and it is of a somewhat porous or spongy nature so that the gasoline quickly penetrates through it and acts on the rubber particles to dissolve, or at least to soften, them. That part of the gasoline which permeates the rubber coating also acts on the Cumar coat and begins to dissolve it. This action proceeds very rapidly so that in a matter of fifteen or twenty seconds the decalcomania film is freed from the backing sheet and can either be slid off or the backing sheet can be peeled off. In either event a clean separation of the backing sheet is produced. It is not strictly correct from a scientific standpoint to say that the rubber particles are dissolved by gasoline, although whether or not this is the fact is not material so far as this invention is concerned. The gasoline, however, does penetrate the rubber coat, it swells the rubber particles, and so far softens or dissolves this and the Cumar coat that the union of the Cumar coat with the backing sheet is substantially destroyed and a high degree of slip or lubrication is produced in place of the adhesion which formerly existed. In addition, the separation of the decalcomania film from the swell-

ing of the rubber particles in the under coating, which has the effect of pushing the film and the backing away from each other.

In making the Cumar composition it is preferable to use the hardest grade of this resin and to make a solution of a fairly high concentration, say 60%. Other gums, however, such as ester gum, can be used instead of part or all of the Cumar, although I have not found it as satisfactory as the latter. By "ester gum" I mean the compound that also goes under the name of rosin ester or glycerinated rosin. Araclor resin can also be used to supplement a part of the Cumar. This resin consists of chlorinated diphenyl and other chlorinated diaryls. A considerable variety of other rubber compounds can also be used in place of the latex. Vulcanized rubber latex can be substituted for the common latex of commerce which, of course, is unvulcanized, and forms a very satisfactory substitute for it. However, it is more expensive and there is no substantial advantage in using it. Also the latex rubber, whether vulcanized or unvulcanized, is definitely superior for the purposes of this invention to milled rubber.

An important advantage of the product above described is that the outer coat is not substantially affected by the more common solvents used in the inks with which the decalcomania designs are printed on this surface. Also, it is a common practice to apply a coating of clear lacquer over a decalcomania design, and the Cumar resin coat is highly resistant to the solvents commonly used in such a lacquer.

In applying decalcomanias of this type to veneer and other water absorbing bodies, some absorption of the solvent may occur, but these solvents are so volatile that they evaporate rapidly and do not produce any warping of the veneer. Consequently, they completely avoid the objection above described to the use of common forms of decalcomanias. As above stated, a considerable variety of these volatile solvents of a hydrocarbon nature are available at reasonable prices so that the expense involved in the use of such a solvent instead of water is not a serious practical objection.

In some cases decalcomania manufacturers prefer to use an ink which, from a chemical point of view, is really a varnish or paint and includes a vegetable oil, or some other constituent which will attack the Cumar coat. When such an ink is to be used I prefer either to substitute for the outer Cumar coat, or to cover it with, an outside coat of some material which will not be affected by an ink of this kind. For this purpose a coating material made of gum sandarac and rosin may be used, the composition consisting of approximately seven parts, by weight, of gum sandarac to ten parts of rosin (colophony), or shellac, dissolved in about nine parts of denatured alcohol as, for example, Formula No. 5 prescribed by the U. S. Internal Revenue Bureau.

It will be evident that the union of the outer coat to the backing sheet need not consist of a single coat having the characteristics above described, the essential point being that a coat or coats having these characteristics be interposed between the outer coat and the backing sheet so that the release of the decalcomania and its separation from the backing sheet will be produced in substantially the manner above set forth.

Having thus described my invention, what I desire to claim as new is:

1. A decalcomania paper comprising a suitable backing sheet, an outer waterproof coating carried by said sheet to take decalcomania printing, and a protective coating of a rubbery nature between the first mentioned coating and said sheet. 5
2. A decalcomania paper comprising a suitable backing sheet, an outer waterproof coating carried by said sheet to take decalcomania printing, and an intermediate coating of a rubbery nature bonding the first mentioned coating to 10 said backing sheet.
3. A decalcomania paper comprising a suitable backing sheet, and a plurality of coatings of waterproof material in superposed relationship 15 on one face of said sheet, said coatings having radically different characteristics, the outermost of said coatings being adapted to take decalcomania printing and one of the coatings being of a rubbery nature.
4. A decalcomania paper comprising a suitable backing sheet, an outer waterproof coating of a resinous nature carried by said sheet to take decalcomania printing, and an intermediate coating of a rubbery nature bonding the first mentioned coating to 20 said backing sheet.
5. A decalcomania paper comprising a suitable backing sheet, an outer waterproof coating of a resinous nature carried by said sheet to take decalcomania printing, and an intermediate coating consisting chiefly of latex rubber bonding the first mentioned coating to said backing sheet. 25
6. A decalcomania paper comprising a suitable backing sheet, an outer waterproof coating carried by said sheet to take decalcomania printing, the predominating constituent of said coating being coumarone-indene resin, and an intermediate waterproof coating bonding the first men- 30
- tioned coating to said backing sheet, the predominating constituent of said intermediate coating being latex rubber. 35
7. A decalcomania paper comprising a suitable backing sheet, an outer waterproof coating carried by said sheet and adapted to take decalcomania printing, said coating being highly resistant to the common solvents used in printing ink, an under waterproof coating of a resinous nature bonded to said outer coating and a third waterproof coating bonding said under coating to said sheet, said third coating containing a substantial percentage of a rubbery constituent and being adapted to be swelled and softened by the action of a non-aqueous solvent, and when so acted upon having a high degree of slip. 40
8. A decalcomania paper comprising a suitable backing sheet, and a plurality of coatings in superposed relationship on one face of said sheet, said coatings having radically different characteristics, the outermost of said coatings being adapted to take decalcomania printing and one of the coatings being of a rubbery nature, said backing sheet being pervious to a liquid solvent for one of said coatings. 45
9. A decalcomania paper comprising a suitable backing sheet, an outer waterproof coating carried by said sheet adapted to take decalcomania printing, and a plurality of additional coatings between said outer coating and said sheet and bonding the outer coating to the backing sheet, said intermediate coatings having radically different characteristics and one of them being of a rubbery nature, said backing sheet being pervious to a liquid solvent for one of said intermediate coatings. 50

LEWIS DAVIS.